

May 16, 1933.

O. M. OTTE

1,909,887

ROLLING IN A MAGNETIC FIELD

Filed July 13, 1932

4 Sheets-Sheet 1



INVENTOR.

By Otho M. Otte  
Green & McCallister  
His ATTORNEYS.

May 16, 1933.

O. M. OTTE

1,909,887

ROLLING IN A MAGNETIC FIELD

Filed July 13, 1932

4 Sheets-Sheet 2



Fig. 2.



Fig. 4.

INVENTOR.  
Otho M. Otte  
BY Green & McCallister  
His ATTORNEYS.

May 16, 1933.

O. M. OTTE

1,909,887

ROLLING IN A MAGNETIC FIELD

Filed July 13, 1932

4 Sheets-Sheet 3



INVENTOR.  
Otho M. Otte  
BY Green & McCallister  
His ATTORNEYS.

May 16, 1933.

O. M. OTTE

1,909,887

ROLLING IN A MAGNETIC FIELD

Filed July 13, 1932

4 Sheets-Sheet 4



INVENTOR.  
Otho M. Otte  
BY  
Green & McCallister,  
Also ATTORNEYS.

## UNITED STATES PATENT OFFICE

OTHO M. OTTE, OF TARENTUM, PENNSYLVANIA, ASSIGNOR OF ONE-HALF TO HARRY F. PORTER, OF BRACKENRIDGE, PENNSYLVANIA

## ROLLING IN A MAGNETIC FIELD

Application filed July 13, 1932. Serial No. 622,335.

This invention relates primarily to magnetic materials and their manufacture and treatment, and incidentally to the treatment of other metallic materials for the production therein of certain desirable characteristics or qualities.

Magnetic materials to which this invention is primarily directed are those used as core materials and include all metals or metal alloys having the characteristics or qualities which render them suitable as core materials.

Other magnetic materials to which this invention is directed are those suitable for use in the make-up of permanent magnets.

While I have directed my studies primarily to magnetic materials, I believe that the underlying method or procedure hereinafter outlined, if utilized in the manufacture or treatment of metallic materials other than magnetic materials, will produce certain desirable qualities or characteristics therein, or at least enhance the value of such materials for use in situations where the maximum of certain qualities or characteristics is desired.

The term "metallic material" as used herein is intended to include metals and metal alloys and particularly ferrous metals and alloys having a ferrous base, but is not intended to exclude other metals or alloys.

Critical temperature range as used herein designates that range of temperatures through which a magnetic material passes when changing from the non-magnetic state to the magnetic state and vice versa, and includes that temperature at which molecular rearrangement within any metal or metal alloy occurs.

The properties of all metallic materials, with which I am familiar, undergo fundamental changes when the material is heated to a temperature well above its critical temperature range and allowed to cool down to a point below said range and it is my belief

that these changes occur because of molecular rearrangement within the material.

At temperatures above the critical temperature range, all metallic materials known to me are non-magnetic. At temperatures below the critical temperature range, many metallic materials are magnetic and the magnetic properties of such materials become more pronounced the lower the temperature of the material.

Hot working, such as rolling or other forging of metallic materials is preferably carried on (at least to a major extent while the material is at a temperature well above its critical temperature range.

This invention fundamentally consists in subjecting metallic materials to the influence of a relatively strong magnetic field and while so influenced in rolling or otherwise forging the same during the period while it is within its critical temperature range. Specifically, the invention consists in rolling or otherwise forging a metallic material throughout a period which starts at a point well above its critical temperature range and continues until the temperature of the material has dropped to a point below its critical temperature range and during such working, in subjecting the material to the influence of a relatively strong magnetic field.

While the treatment thus broadly described is applicable to the manufacture and/or finishing of various metals and metal alloys I am primarily interested in magnetic materials used in certain parts of electrical apparatus having alternating magnetic fields such as transformer cores, armature cores, pole pieces and magnetic poles of various kinds. These are preferably or necessarily of laminated structure and sheets or plates therefore are usually employed in building up the same.

The material used for transformer cores and to a lesser extent that used in alternating current generators must be characterized

by low hysteresis loss. In transformer cores especially, the hysteresis loss is of most important consideration but it is desirable to combine low hysteresis loss with high permeability. It is desirable to have the material for these uses pliable and free from brittleness.

An object of this invention is the provision of a method of improving metallic materials for use as magnetic materials.

10 Another object of this invention is the provision of a method of manufacture for or treatment in the production of magnetic materials either in the form of sheets or plates for use in the make-up of parts of electrical apparatus or as permanent magnets for which latter use the material will not be in the form of laminae, whereby such materials are greatly improved for the uses to which they are to be put.

20 A still further object of this invention is the provision of a method of treatment whereby finished or semi-finished sheets or plates of magnetic material such as silicon steel may have their watt-loss values materially decreased below the values of the best magnetic material manufactured today and with which I am familiar.

30 A still further object of this invention is the provision of a method whereby desirable characteristics or qualities of alloys in the form of sheets, plates, tubes, bars, wire, etc., may be obtained therein without affecting the material of such products in any undesirable manner.

35 A still further and more limited object of this invention is to provide a method whereby the resistance to corrosion of certain alloys may be increased. Some of these alloys are known to the trade as "Allegheny Metal", "KA-2", "18-8" and "Enduro".

40 These as well as other objects which will appear to those skilled in the arts to which this invention relates, I attain by means of the method or treatment or processing broadly described above and hereinafter specifically described in connection with the manufacture of sheet material and that for use in making up permanent magnets.

50 Since the method of my invention broadly consists in performing work (such as rolling or forging) on a metal or metal alloy while the same is lowering in temperature from a temperature above the point or range at which molecular rearrangement therein occurs to a temperature below such point or range and while subjected to the influence of a relatively strong magnetic flux or field, it (the method) is capable of being carried out in numerous ways.

55 Since standard methods of hot rolling or forging and standard apparatus for heating the material and working, rolling or hammering the same, as the case may be, can be utilized, it is only necessary to provide the

relatively strong magnetic field and to so correlate the same to the rolls or hammer and the work done thereby (such as reducing the gauge of partially finished sheet or plate material or the finishing of a forging or obtaining the final pass in a bar mill or tube mill) that such work takes place within such magnetic field, or so nearly adjacent thereto that the material being hot worked is beneficially influenced by said field or flux.

60 In order that a complete understanding of my invention in connection with certain types of hot working may be had, I have included certain drawings in this application which more or less schematically illustrate certain apparatus by means of which the method of my invention may be carried into effect.

65 For instance, I have illustrated a two-high finishing mill equipped for subjecting to the influence of a relatively strong magnetic field, packs of semi-finished magnetic sheet material.

70 I have also schematically illustrated two stands of a strip finishing mill equipped for practicing my method as well as a hammer for performing forging operations and equipped for carrying out my method. In the drawings:

75 Figure 1 is a view in front elevation of a two-high finishing mill equipped for carrying out my invention;

80 Fig. 2 is a view in end elevation of said mill as seen looking from right to left in Fig. 1;

85 Fig. 3 is a more or less diagrammatic view and represents the reducing rolls of two stands arranged in tandem adapted for the rolling of strip material and being equipped for the practice of my invention;

90 Fig. 4 is a view in front elevation looking toward the entrance side of one of the pair of rolls embodied in the two stands of Fig. 3;

95 Fig. 5 is a more or less diagrammatic view illustrating a pair of reducing rolls and the mechanisms for feeding material to and from a pair of rolls equipped for the practice of my invention; and

100 Fig. 6 is a pictorial view illustrating a forging hammer so equipped as to be suitable for the practice of my invention upon forgings.

105 When plates or sheets are to be rolled or finished in accordance with my invention, I may use apparatus such as that disclosed in Figs. 1 and 2, wherein is disclosed a two-high mill, generally of conventional type, suitable for rolling or finishing either sheet packs or plates as the case may be.

110 It is in the finishing pass or passes that I preferably utilize my invention, because it is in these passes where the benefits derived from the method of my invention are most pronounced.

115 When practising the method in the finishing pass or passes in the rolling of either

sheets or plates, the plates or packs are raised, as is now ordinarily done, to rolling temperature, that is, a temperature above the critical temperature range of the material.

5 The apparatus of Figs. 1 and 2 comprises a mill housing made up of the customary parts 10 and 11, each provided with the customary window 12, roll neck brasses 13 and 14 mounted within the windows and rolls 10 15 and 16.

The roll neck brasses being non-magnetic, provide and maintain substantial air gaps between the roll necks and the mill housings, thus largely confining the magnetic flux before referred to within the rolls, the necks and the material being worked on by the rolls.

In such a two-high mill which is ordinarily of the jump variety, the lower roll is the driven roll and in the case of the mill illustrated in Figs. 1 and 2, a non-magnetic coupling member 17 is provided for connecting the roll neck end 18 to a driving spindle (not shown).

Since a relatively strong magnetic field or flux is desirable for influencing the material being rolled, I preferably provide two relatively powerful electromagnets so as to obtain two co-operating magnetic fields and through which the material being worked on or rolled passes during the period of roll reduction.

Each of these electromagnets has a generally horseshoe-shaped core 20 which may be solid if direct current is to be used for energizing the same and laminated if alternating current is to be used for this purpose.

Each magnet is provided with a suitable winding 21 adapted to be connected to a source of supply of electric current (not shown). The lower leg of each magnet is formed so as to provide a snug sliding fit with the extended cylindrical end 22 of the lower roll 16. The portions of the magnet core or rather the end of the lower leg of each magnet is split as shown at 23 in order that the magnets may be readily assembled on the extended necks of the lower roll 16.

Since the upper roll is so mounted as to be capable of jumping or rising above the lower roll when material enters the pass between the rolls, the upper legs 24 of the magnets are provided with side faces 25 which are flat and smooth and are adapted to bear against the smooth, flat ends 26 of the roll necks of upper roll 15.

While an appreciable distance is shown in Fig. 1 of the drawings between the ends of the necks of roll 15 and the adjacent faces 25 of the upper legs of the electromagnets, this distance in actual practice is made as small as possible and in fact a metal to metal contact, plus the necessary oil film, which is preferably and normally maintained to reduce friction caused by the pull of the magnets on the roll necks of both rolls. In practice, the ends

of the magnets are preferably water cooled whereby no appreciable heat is transferred from magnet to rolls or vice versa.

Each magnet is preferably mounted in place by means of a laterally extending support foot 27, a support base 28 and a roller fulcrum 29. Such a structure minimizes the sliding friction between the bore of the lower legs of the magnets and the extended necks 22 of lower roll 16; the position of laterally extending support foot 27 being chosen with this end in view.

Lifting eyes 30 are preferably provided whereby the magnets may be readily transported from place to place and located in operative position with relation to the reducing rolls.

The roll necks, as is now common, are preferably furnished with an adequate supply of water through pipes 31 controlled by valves 32.

The mechanisms more or less diagrammatically disclosed in Fig. 5 are adapted to permit magnetic material to be fed through the roll pass and to scrape from the rolls any material which may adhere thereto.

The material being reduced by the rolls 15 and 16 is marked 33 and in the set-up illustrated in Figs. 1 and 2, the magnetic field or flux lines created by the two electromagnets are indicated by the arrows. It will be seen that when the magnets are arranged as in Figs. 1 and 2, the magnetic lines pass perpendicularly through the material being rolled.

In Fig. 5, as before stated, I have schematically illustrated mechanisms for guiding material to and from the reducing rolls of a mill. Such mechanisms with suitable modifications can be used for either a two-high finishing mill or a strip mill of either the two, three, or four-high variety.

As in Fig. 5, I may employ a frame 34, which supports a fore table 35 made of non-magnetic material and a cover 36 preferably upwardly curved at its entrance side as at 37. The table and cover are preferably provided with scrapers 38 and 39 yieldingly held in contact with the upper and lower reducing rolls respectively, by some means, such as springs 40 and 41. Cover 36 is preferably provided with a top member 42 which is secured at its forward end as at 43 to cover 36 and adjacent its rear end rests on an upward extension 44 of frame 34.

At the outlet side of the rolls, strippers 45 and 46 are employed and these are preferably formed with angled arms, as shown in Figure 5, whereby they are yieldingly held in contact with the rolls by means of springs 47 and 48. The material leaving the rolls 15 and 16 passes between non-magnetic members 49 and 50.

The material being rolled is designated 33 as in Fig. 1 and may either be semi-finished packs, or semi-finished strip or plate ma-

terial. The mechanisms of Fig. 5 are adapted first to feed the material to and from the reducing rolls and to prevent it from curling around the rolls due to magnetic pull 5 during the roll reduction, next, to keep the reducing rolls stripped free from adhering particles of material, and next to strip the material from the rolls as is now common.

Member 49 is provided with an inclined 10 guide member 51. Guide members 42 and 51 are useful in connection with a two-high finishing mill either when operated by hand or by means of a mechanical manipulator as they serve to guide the material over the top 15 roll in passing back from the catcher side of the mill to the roller side of the mill.

In Figs. 3 and 4, I have shown my invention applied to two stands arranged in tandem such as employed in continuous rolling. 20

When my invention is employed in connection with two stands arranged in tandem, the magnetic field set-up in the material during its reduction is disposed along or with the grain of the material, that is, longitudinally 25 of the piece as is clearly indicated in Fig. 3, for example.

In this form of the invention, I suitably connect the laminated or solid cores 52 to successive pairs of rolls 53 and 54 and provide 30 said cores with suitable windings 55. In this way, the magnetic field instead of traversing the piece across or perpendicularly to the grain as in Figs. 1 and 2 follows along the grain in the longitudinally set-up magnetic 35 field through the core above the piece 33 and through the core below it. Consequently, assuming that the material is traveling in the direction of the arrow (Fig. 3) the lower magnetic field traverses the lower core longitudinally and passes into the forward lower 40 roll and upwardly to the piece and thence along the piece rearwardly to the lower roll behind and thence downwardly into the core again. Above the piece, the field passes along 45 the core, into the upper roll 53, down into the piece, along the piece rearwardly to the roll behind and thence upwardly into the upper roll 54. In both Figs. 3 and 4 the arrows 50 represent the direction of the field. In the case of tandem mills no special supporting 55 means for the cores are required. The ends of the core pieces may be provided with suitable holes 57 which suitably receive the roll necks 58. The equivalent of an air gap may be maintained between the roll necks and the supporting framework 59 by non-magnetic 60 bearings or brasses 60 as will be understood.

In Fig. 6, I have illustrated a further application 60 of the principles of my invention in connection with a forge, press or other suitable piece of apparatus. Whatever may be the practice, form or use of the apparatus it is preferably supported on the nonmagnetic base 61 and intermediate its frame-

work a suitable core 62 is interposed which is provided with windings 63 in the usual way and as will be understood from the foregoing. 64 represents the material being operated upon and as indicated by the arrows the magnetic field passes along the core into the framework of the machine, downwardly thereafter and through the material being operated upon and then back through the framework to the core by the shortest and easiest path as is characteristic of magnetic fields.

While my invention is particularly applicable to the finishing of sheet, plate or strip material, it will be apparent that it may also be utilized in the finishing of rods, bars, tubes, wire and the like.

It is not necessary that the method of my invention be utilized in the standard mill practice of finishing sheets, strips or plates, but if desired, finished sheets, strips or plates may be treated in accordance with this invention and in the case of finished sheets, it is preferable to apply the method to two, three or four sheets. These may be placed as in a pack, raised to the proper temperature and then given one or more passes with 90 in the magnetic field. The reduction made on the finished sheets may be only slight, if 95 desired.

I find that in some cases a material advantage is obtained even if the material being treated is not raised to a temperature above the critical range for such material. In fact, the material may be treated cold or at room temperature or above. In some cases, the reduction made in the pass or passes wherein the material is subjected to the magnetic flux, may be as slight as 1% or 100 from 1% to 3%.

I find that advantages are obtained where the material is stretched as by means of a stretcher leveler during the time it is subjected to the action of magnetic field.

Due to the tendency of the reducing rolls to move one toward the other under the influence of the magnetic pull, the mill housings are relieved of a material amount of strain and the spring of the rolls is materially lessened.

I believe that I will be able to maintain a much flatter pass than has been possible heretofore and for this reason, I believe that magnetic sheets rolled in accordance with this invention will be much more uniform as to magnetic and electrical properties than sheets heretofore made.

Having thus described my invention, what I claim as new and desire to secure by Letters Patent is:—

1. A method of improving characteristics of a metallic material, which consists in heating the material to a temperature above that at which molecular rearrangement therein occurs and then mechanically working said

- material while cooling from said temperature to a temperature below the point at which such rearrangement occurs and, while so mechanically working, in subjecting said material to the influence of a magnetic field of such intensity as to contribute to such improvement.
2. A method of improving the magnetic properties of a metallic material, which consists in heating the material to a temperature above that at which molecular rearrangement therein occurs and then prior to rearrangement in subjecting said material to pressure sufficient to change the cross section thereof and while subjected to such pressure in subjecting said material to the influence of a magnetic flux of sufficient intensity to contribute to improvement of the material.
3. A method of improving the magnetic characteristics of metallic sheeted material, which consists in heating the material to a temperature above that at which molecular rearrangement occurs within the material, then in reducing the gauge of the sheeted material at about the time such molecular rearrangement occurs and during such reduction in gauge in subjecting the material to the influence of a magnetic flux of sufficient intensity to beneficially influence the magnetic characteristics.
4. A method of obtaining desired characteristics in silicon steel sheets which consists in carrying on the final reduction at that temperature where molecular rearrangement within the material occurs and during such reduction in subjecting the material to the influence of a magnetic flux of sufficient intensity to beneficially influence the magnetic characteristics.
5. A method of finishing magnetic sheets which consists in completing the final mechanical reduction of a pack at a temperature not lower than the ordinary re-heating temperature, and while making such reduction in subjecting the pack to the influence of a relatively strong magnetic flux.
6. A method of finishing magnetic sheets which consists in completing the final mechanical reduction of a pack at a temperature not lower than the ordinary re-heating temperature, and while making such reduction in causing a magnetic flux of relatively great intensity to traverse the pack on lines perpendicular thereto.
7. A method of beneficially affecting the grain structure of ferrous material reduced to form by rolling or other forging which consists in heating the material to be rolled or forged to a temperature above that at which molecular rearrangement within the material occurs, in subjecting the heated material to the influence of a traversing magnetic flux of relatively great intensity and in performing the rolling or forging prior to and during the time the material drops below the temperature of molecular rearrangement and while the same is under the influence of said magnetic flux.
8. A method of improving characteristics of a metallic material, which consists in mechanically working said material while at about the temperature at which molecular rearrangement therein occurs and while so working in subjecting said material to the influence of a magnetic field of such intensity as to contribute to such improvement.
9. A method of improving the magnetic properties of a metallic material, which consists in subjecting said material to pressure sufficient to change its cross sectional area while said material is at about the temperature at which molecular rearrangement takes place and while such material is subjected to the influence of a magnetic flux of sufficient intensity to influence the molecular rearrangement.
10. A method of improving characteristics of a metallic material, which consists in heating the material to rolling temperature, in mechanically working the material and in subjecting the same to the influence of a magnetic field of such intensity as to contribute to such improvement.
11. A method of improving the magnetic properties of a metallic material, which consists in heating the material to rolling temperature, then in subjecting said material to pressure sufficient to change the cross section thereof and while subjected to such pressure in subjecting said material to the influence of a magnetic flux of sufficient intensity to contribute to improvement of the material.
12. A method of improving the magnetic characteristics of metallic sheeted material, which consists in heating the material to rolling temperature, then in reducing the gauge of the sheeted material and during such reduction in gauge in subjecting the material to the influence of a magnetic flux of sufficient intensity to beneficially influence the magnetic characteristics.
13. A method of obtaining desired characteristics in silicon steel sheets which consists in carrying on the final hot reduction within the influence of a magnetic flux of sufficient intensity to beneficially influence the magnetic characteristics.
14. A method of finishing magnetic sheets which consists in completing the final mechanical reduction of a pack while the same is subjected to the influence of a relatively strong magnetic flux.
15. A method of finishing magnetic sheets which consists in completing the final mechanical reduction within a magnetic flux of relatively great intensity and traversing the pack on lines perpendicular thereto.
16. A method of improving characteristics of a metallic material, which consists in me-

- chanically working said material while hot and while so working in subjecting the same to the influence of a magnetic field of such intensity as to contribute to such improvement.
- 5 17. The method of producing changes in metallic materials that enhance the properties thereof, that comprises mechanically working the material while hot and being subjected to magnetizing forces of such intensity 10 as to permeate the same with magnetic lines of force.
18. The method of producing changes in metallic materials that make for improvement in the general properties thereof and 15 pronounced improvement in certain specific properties that comprises mechanically working the material while hot and being subjected to magnetizing forces.
19. The method of producing changes in 20 metallic materials that enhances the properties thereof, that comprises mechanically working the material, as by rolling or forging, while hot and being subjected to magnetizing forces.
20. The method of producing changes in 25 metallic material that make for improvement in the quality of its properties that comprises mechanically working the material, as by rolling or forging, and applying magnetizing forces to the material in such manner as 30 to permeate the material with magnetic lines of force at the points where the mechanical forces are applied.
21. The method of improving the physical 35 and/or magnetic properties of metallic materials that comprises heating the material to a temperature such that the material will take a predetermined amount of elongation, placing the material within a magnetic field, and 40 elongating the material while in said field.
22. The method of improving the physical and/or magnetic properties of metallic materials that comprises heating the material to a temperature within the range at which 45 molecular rearrangement occurs, placing the material in a magnetic field, and mechanically stressing the material while in said field.
23. The method of improving the physical and/or magnetic properties of metallic materials that comprises heating the material to a temperature above that at which molecular rearrangement occurs, placing the material within a magnetic field and stressing the material beyond the yield point thereof.
- 55 24. The method of improving the physical and/or magnetic properties of paramagnetic materials that comprises heating the material to a temperature within the range defined by the decalescent and recalescent points of the 60 material, mechanically stressing the material while within said temperature range to produce a permanent set therein, and magnetizing the material in a direction normal to the direction of stress.
- 65 25. The method of improving the physical and/or magnetic properties of metallic materials that comprises deforming the material by mechanically stressing the material, and subjecting the material to the action of a magnetic field while under stress. 70
26. The method of improving the physical and/or magnetic properties of metallic materials that comprises heating the material, placing the material within a magnetic field, and elongating the heated material while in 75 said field.
27. The method of improving the physical and/or magnetic properties of metallic materials that consists in producing beneficial rearrangement of the molecular structure of the material by subjecting the material to the action of mechanical and magnetizing forces of sufficient magnitude to effect such rearrangement. 80
28. The method of improving the physical and/or magnetic properties of paramagnetic materials that comprises heating the material to a temperature within the range defined by the decalescent and recalescent points of the material, mechanically stressing the material while within said temperature range to produce a permanent set therein, magnetizing the material in a direction normal to the direction of stress, and allowing the material to cool while being so stressed and magnetized. 85
29. The method of producing electrical sheets each having substantially the same watt loss, per unit of weight, resulting from varying and/or periodic magnetizing forces, that comprises hot rolling a starting piece through the usual number of reducing and finishing passes, cutting the rolled material into strips or sheets, placing the sheets in a magnetic field and stressing to the point of 90 producing a permanent set therein while in said field. 100
30. The method of producing electrical sheets each having substantially the same watt loss, per unit of weight, resulting from varying and/or periodic magnetizing forces, that comprises hot rolling a starting piece through the usual number of reducing and finishing passes, cutting the rolled material into strips or sheets, placing the sheets in a magnetic field and stressing said sheets beyond the yield point thereof while in said field. 105
31. The method of producing electrical sheets each having substantially the same watt loss, per unit of weight, resulting from varying and/or periodic magnetizing forces, that comprises hot rolling a starting piece through the usual number of reducing and finishing passes, cutting the rolled material into strips or sheets, heating said sheets to a temperature above that at which decalescence occurs, placing said sheets in a magnetic field, and then mechanically stressing the sheets to 110 or beyond the yield point. 120
- 115
- 125
- 130

32. The method of producing electrical  
sheets each having substantially the same  
watt loss, per unit of weight, resulting from  
varying and/or periodic magnetizing forces,  
5 that comprises hot rolling a starting piece  
through the usual number of reducing and  
finishing passes, cutting the rolled material  
into strips or sheets, heating said sheets to a  
temperature above that at which decalescence  
10 occurs, placing said sheets in a magnetic field  
and stressing said sheets in tension sufficient  
to produce elongation therein.

In testimony whereof, I have hereunto sub-  
scribed my name this 8th day of July, 1932.

15 OTHO M. OTTE.

20

25

30

35

40

45

50

55

60

65